

# UNITED STATES PATENT OFFICE.

CHARLES M. STINE, OF WOODBURY, NEW JERSEY, ASSIGNOR TO E. I. DU PONT DE NEMOURS AND COMPANY, OF WILMINGTON, DELAWARE, A CORPORATION OF DELAWARE.

## BLASTING-CAP CHARGE.

1,309,552.

Specification of Letters Patent. Patented July 8, 1919.

No Drawing.

Application filed August 12, 1916. Serial No. 114,498.

To all whom it may concern:

Be it known that I, CHARLES M. STINE, of Woodbury, in the county of Gloucester, and in the State of New Jersey, have invented a certain new and useful Improvement in Blasting-Cap Charges, and do hereby declare that the following is a full, clear, and exact description thereof.

My invention relates particularly to charges to be inserted in blasting caps so as to explode main charges of any suitable type.

The object of my invention is to provide an explosive charge adapted for use in blasting caps and in different types of primers used for the detonation of high explosives. More particularly the object of my invention is to provide an explosive charge suited for use in blasting caps or in primers of other types, said charge containing a compound which contains both a nitro group and a nitrate group.

While my invention is capable of embodiment in many different forms for the purpose of illustration I have described only certain forms thereof hereinafter.

For example, my invention may be carried out as follows:

A blasting cap made in accordance with my invention may contain any explosive compound which contains a nitro and a nitrate group, but, for example, it may contain any one of the compounds represented by the following formulæ:



40 These compounds may be prepared in any suitable way, but I have described one way of manufacturing the same in my co-pending application upon "Process of producing explosive compounds, and product thereof", Serial No. 110278, filed July 20, 1916.

45 These compounds are very highly explosive, and are easily detonated by a very small amount of priming material, as, for example, fulminate of mercury or lead azid.

50 For example, dinitrotolylene nitrate,



produces in this way a very powerful blasting cap charge or composition. A blasting cap may be provided with from 0.4 to 1.0 gram of dinitrotolylene nitrate, the amount 55 used depending upon the grade of blasting cap desired. This is pressed into the copper shell of the cap in the usual manner. On top of this there is pressed a priming charge consisting of about 0.4 gram of 60 mercury fulminate. Instead of placing the dinitrotolylene nitrate and the fulminate of mercury in separate layers, these two compounds may be mixed together, for example, in the proportion of 80 parts dinitrotolylene nitrate to 20 parts fulminate of 65 mercury, and the mixture pressed into a copper shell. This produces a very powerful blasting cap which when ignited by the ordinary safety fuse or by electrical 70 means or otherwise provides an exceedingly efficient agent for the detonation of dynamite or other high explosive.

While I have described my invention above in detail, I wish it to be understood 75 that many changes may be made therein without departing from the spirit of my invention. For example, I do not desire to limit myself to any particular method of producing the above compounds, nor to any 80 particular proportion thereof, nor to any particular manner of using the same.

I claim:—

1. An explosive composition containing an organic compound having therein a nitro group and a nitrate group, and a priming material. 85
2. An explosive composition containing an organic compound of the aromatic series having therein a nitro group and a nitrate group, and a priming material. 90
3. An explosive composition containing an organic compound having therein a nitro group and a nitrate group, and a priming material, there being a plurality of one of 95 said groups present.
4. An explosive composition containing an organic compound of the aromatic series having therein a nitro group and a nitrate group, and a priming material, there being 100 a plurality of one of said groups present.
5. A priming composition containing an

organic compound of the aromatic series having the formula:



- 5 6. A priming composition comprising a dinitrotolyene nitrate and fulminate of mercury.
7. A priming composition comprising 80

parts dinitrotolyene nitrate and 20 parts of fulminate of mercury.

10 In testimony that I claim the foregoing I have hereunto set my hand.

CHARLES M. STINE.

Witnesses:

FRANK L. POTE,  
WM. G. LODGE.